

# UNITED STATES PATENT OFFICE.

JACOB S. ROBESON, OF CAMDEN, NEW JERSEY, ASSIGNOR TO ROBESON PROCESS COMPANY, OF CAMDEN, NEW JERSEY, A CORPORATION OF NEW JERSEY.

## COMPOSITION OF MATTER AND PROCESS OF MAKING SAME.

No. 851,379.

Specification of Letters Patent.

Patented April 23, 1907.

Application filed May 10, 1906. Serial No. 316,129.

*To all whom it may concern:*

Be it known that I, JACOB S. ROBESON, a citizen of the United States, and a resident of Camden, Camden county, New Jersey, have 5 invented an Improved Composition of Matter and Process of Making the Same, (Case B,) of which the following is a specification.

My invention relates to compositions of matter having adhesive properties, and consists of an improved compound of this nature comprising a mass of sulfite liquor combined with a soluble albuminoid.

My invention comprises further the method or process of making this improved composition of matter.

In the manufacture of cellulose or paper pulp under what is known as the "sulfite process," which consists in boiling wood and other fibres under pressure in a solution containing sulfurous acid and a base, such as lime or magnesia, a vast quantity of a watery mixture known as "waste sulfite liquor" is produced that hitherto has had little value, besides being highly objectionable in a number of ways and very difficult of disposal. In carrying the method or process of my present invention into effect, I employ a concentrated or evaporated solution of the same; preferring to use a neutral, undecomposed and concentrated mass of this waste liquor made in accordance with a method I have developed for utilizing such material. In my patent, No. 833,634, dated October 16, 1906, I have set forth a process of treating this raw waste liquor, by rendering it substantially neutral with the aid of milk of lime or other suitable alkaline material, and then quickly concentrating such neutralized body *in vacuo*, without decomposition, to a desirable density. In the preferred method or process of making my improved compound, I propose to use this substantially neutral, undecomposed and concentrated mass of sulfite liquor made in accordance with the process above set forth, and to a quantity of this liquor at a density of about 25° B., I add a small quantity of a solution of a soluble albuminoid, for instance, any of the well-known forms of animal glue, and incorporate the

50 glue with the concentrated sulfite liquor by stirring or other suitable agitation with or without heat. As another instance of a soluble albuminoid for admixture with the sul-

fite liquor, I may mention that packing house product or residue, familiarly known as concentrated tankage or "stick." In the manufacture of fertilizers from waste animal matter, the water with which such material has been cooked to separate the fat, becomes impregnated more or less therewith and also 60 with a large quantity of nitrogenous material. It is technically known as tank water and is the source of concentrated tankage, or "stick," which is made by evaporating said tank water. The density of the sulfite liquor 65 may vary within certain proportions, but approximately should not be less than 14° B., and may range as high as 40° B.

The solution of soluble albuminoid, for instance any of the well-known forms of animal 70 glue, is preferably in the proportion of about 10 per cent by weight of the water used; that is to say, about two ounces of glue are to be dissolved in twenty ounces of water. This proportion, however, is only approximate, as it may vary with the character of the glue used, and in some experiments, presumably with a weaker glue I have used as 75 much as four ounces of glue with twenty ounces of water.

I have discovered that the substantially neutral and undecomposed mass of sulfite liquor made in accordance with the process above referred to, throws down no precipitate upon the addition of glue, and, hence, 85 my process differs widely from the prior practice in the art to which my invention relates, and in which various compounds comprising sulfite liquor and glue are disclosed. The formation of a precipitate by the addition of glue to sulfite liquors heretofore treated appears to be well recognized, and the commonly accepted method of preventing the formation of such precipitate is to change the character of the sulfite liquor, 90 whether in the raw or concentrated state, before the addition of the glue. The neutral mass which I employ, however, requires no change other than the necessary evaporation according to my process above set forth, and 100 numerous experiments carried out at various temperatures and at various degrees of density within the range noted, indicate clearly that no precipitate is thrown down.

In practice, I have found that a mixture 105 consisting of five parts by volume of the neu-

tral and concentrated mass of waste sulfite liquor and one part by volume of a solution of a soluble albuminoid, animal glue, for instance, gives uniformly satisfactory results.

5 I do not wish, however, to be understood as limiting myself to the employment of these ingredients in the proportions given, but I believe they are the best adapted to give good results.

10 The composition of matter made in accordance with my invention is in liquid form and may be employed as an adhesive or as a sizing compound. When "stick" is employed as the soluble albuminoid, the material resulting from such combination is valuable as a fertilizer.

I claim:

1. A soluble composition of matter forming an adhesive, containing chemically unchanged sulfite liquor, and a soluble albuminoid.

2. A soluble composition of matter forming an adhesive, comprising a mass of concentrated and chemically unchanged sulfite liquor, and a soluble albuminoid.

25 3. A soluble composition of matter forming an adhesive, comprising a substantially neutral, undecomposed and concentrated mass of sulfite liquor, and a soluble albuminoid.

4. A soluble composition of matter forming an adhesive, containing chemically unchanged sulfite liquor, and animal glue.

5. A soluble composition of matter forming an adhesive, comprising a concentrated 35 and chemically unchanged mass of sulfite liquor, and animal glue.

6. A soluble composition of matter forming an adhesive, comprising a substantially neutral, undecomposed and concentrated 40 mass of sulfite liquor, and animal glue.

7. A soluble composition of matter forming an adhesive, comprising five parts by volume of concentrated and chemically unchanged sulfite liquor, and one part by volume of a solution of a soluble albuminoid.

45 8. A soluble composition of matter forming an adhesive, comprising five parts by volume of a substantially neutral, undecomposed and concentrated mass of sulfite liquor, and one part by volume of a solution of animal glue.

In testimony whereof, I have signed my name to this specification, in the presence of two subscribing witnesses.

JACOB S. ROBESON.

Witnesses:

C. A. RAPALLO,  
L. H. WADDROP.